

# UNITED STATES PATENT OFFICE.

WILLIAM HYLAND, OF NEW HAVEN, CONNECTICUT.

## ART OF DECORATING GLASS.

SPECIFICATION forming part of Letters Patent No. 313,671, dated March 10, 1885.

Application filed December 6, 1884. (Specimens.)

*To all whom it may concern:*

Be it known that I, WILLIAM HYLAND, a citizen of the United States, and residing at New Haven, in the county of New Haven 5 and State of Connecticut, have invented certain new and useful Improvements in the Art of Decorating Glass; and I do hereby declare that the following is a full, clear, and exact description of the invention, which will enable others skilled in the art to which it appertains to make and use the same.

This invention relates to improvements in decorating glass or other transparent articles, the object of the same being to increase the 15 brilliancy and luster of the decoration; and it consists in painting or printing of the required design upon the back of the article to be decorated, which is then colored with suitable transparent lacquer-colors, the back of 20 said colored design then being provided with a reflectent metal backing, as and for the purpose hereinafter fully set forth and claimed.

To perform my improved process of decorating glass, &c., I first place upon the back 25 of the article desired to be decorated an outline of the required design, also the necessary shade-lines, as shown in specimen 1, which may be performed either by painting, printing, or any of the numerous modes now 30 in vogue for doing the same. I then fill in the outline of said design with appropriate colors, which consist of colored lacquer, as shown in specimen 2. I prefer the use of colored lacquers, as they are free from the many 35 opaque particles with which other pigments abound, permitting a better reflection of the light through the colored surface. I then apply to the back of the colored design only a coating of bright reflectent metal, as shown in 40 specimen 3, upon which the rays of light are reflected back through the colored design. The design being placed directly upon the glass without any intervening "transferring-varnishes," a beautiful, clear, and brilliant effect 45 is obtained.

Any of the numerous protecting media may be applied, as shown in specimen 4; but it is not essential to achieve the object sought in my invention, as will be readily seen by reference to the specimens.

I am aware that a bright metal has been used as a backing or reflector in "decalcomanie" or transfer decorations; but as they must needs be composed of "oil-colors" which are more opaque than the colored lacquer, 50 there is not the brilliancy and luster to the decoration by their use as that obtained by my improved process. Again, it is necessary in the use of decalcomanie or transfer process to interpose a coating of varnish or 55 size between the design and the glass in order to make the same adhere to the glass, which is dispensed with in my process, thereby bringing the design into clearer view.

I am aware that the painting or printing of 60 a design upon the back of the glass is not new, also that colored lacquers have been used in decorating glass; therefore I do not broadly claim them separately as my invention; but, as far as I am aware, they have never 65 been employed together in a decorating process as hereinbefore described.

What I claim as new, and desire to secure by Letters Patent, is—

As a new process for decorating glass and 70 other transparent articles, consisting of, first, painting or printing an outline design having required shade-lines upon the back of the article to be decorated; second, that of filling in said outlined design with appropriate colored lacquers; third, by coating the back of 75 said colored design with a bright reflectent metal, all being arranged and combined substantially as and for the purpose set forth.

In testimony whereof I affix my signature in 80 the presence of two witnesses.

WILLIAM HYLAND.

Witnesses:

DANIEL CARROLL,  
JOHN H. BARLOW.